

# UNITED STATES PATENT OFFICE.

GEORGE WELLINGTON MILES, OF BELMONT, MASSACHUSETTS.

## METHOD OF MAKING EMULSIONS OF COMPOUND WAXES AND THE PRODUCT OF SAID METHOD.

1,224,948.

Specification of Letters Patent.

Patented May 8, 1917.

No Drawing.

Application filed July 21, 1915. Serial No. 41,176.

To all whom it may concern:

Be it known that I, GEORGE WELLINGTON MILES, a citizen of the United States, and resident of Belmont, in the county of 5 Middlesex and State of Massachusetts, have invented new and useful Improvements in Methods of Making Emulsions of Compound Waxes and the Product of Said Methods, of which the following is a specification.

This invention consists in a method of making emulsions of compound wax comprising paraffin wax and hard wax and in the product of the method.

As stated in my United States Patent No. 1,168,534, dated January 18, 1916, paraffin wax will not respond to methods of emulsification used for other waxes, and this is true whether an emulsion is desired of 20 paraffin wax alone or admixed with other waxes, wax-like substances, or fat acids.

For such purposes as giving to paper a very high gloss or finish, emulsions of hard waxes, such as carnauba wax, Montan wax, 25 shellac wax, Japan wax, are employed, but their high price opposes a strict limitation on their employment.

I have discovered that by melting a relatively small proportion of such a hard wax with a relatively large proportion of paraffin wax, a wax compound is produced which has a melting point close to the relatively high melting point of the hard wax ingredient. The possession of the high 35 melting point renders the compound wax nearly if not quite as effective for paper-finishing purposes as the hard wax ingredient itself.

The paraffin wax in such wax-mixtures does not emulsify in soap solution of the 40 usual degree of dilution. With any ordinary soap there is a critical water proportion, much less than that employed for the emulsification of other waxes, which determines the emulsification of paraffin wax. Such critical water-proportion has to be 45 determined empirically for any given soap.

My method of emulsifying a wax-mixture containing paraffin wax and one or more of 50 the waxes above mentioned, or other hard wax, consists generally in making a soap solution with water in excess of the critical proportion required for the emulsification of the paraffin wax in the mixture; then

mixing the soap solution or paste with the 55 wax-mixture and evaporating the excess water by heat, and beating the mixture. Until the critical water proportion is reached, the paraffin wax in the mixture will not emulsify; but after the requisite 60 reduction of the water, the entire compound wax goes into emulsion.

As a specific example of the method, take a wax-mixture containing, say 75% of paraffin wax and 25% of carnauba wax, or 65 Montan wax, or other hard wax, or more than one kind of other wax. Make a tallow chip soap amounting to 10% by weight of the wax-mixture, a paste or solution, using four or five times its weight of water. Then 70 melt the wax-mixture and stir in the soap paste; heat approximately to the boiling point of water, and continue the heat, stirring or beating, until, by evaporation, the water is reduced to the critical proportion. Thereupon, the entire compound wax 75 emulsifies.

The emulsion thus produced does not behave as a mixture of two distinct waxes, but as an emulsion of a compound wax. 80 The melting point of the wax mixture is quite close to that of carnauba wax alone and this characteristic persists in the wax in emulsion. Consequently, the application of heat (as in paper coating and finishing) 85 does not melt one part of the compound more quickly than another; the relatively high melting point, considerably higher than that of paraffin wax alone, must be attained, and when attained, the emulsified 90 compound wax melts and produces the desired finish.

If the ratio of soda soap to wax, is varied, the critical water proportion will also vary 95 to some extent. The exact limit of this critical proportion cannot be determined, but whatever the soap used, the critical proportion of water will be such that if mixed with the soap alone, it will form a thick viscous paste.

After forming the thick emulsion as above described it may be advantageously extended by the addition of more water.

The mixture of paraffin and other waxes might contain also other ingredients without departing from the invention. It will be understood also that the proportions of 105 paraffin and other waxes might be varied

considerably from the proportions above suggested, and that the invention is applicable to wax mixtures containing any substantial amount of paraffin wax down to 5 20% or even 10% of the whole mixture.

The invention in its broader aspects is applicable generally to emulsifying wax mixtures containing a substantial amount of paraffin wax, whether the other ingredients be other waxes or fat acids, and such 10 broad application of the invention is contemplated by certain of the claims.

I claim:

1. The method of making emulsions of 15 compound waxes comprising paraffin wax and a relatively hard and high melting wax, which consists in melting the ingredient waxes together to form the compound wax, and then heating the wax mixture with soap 20 and a quantity of water appropriate to the emulsification of the paraffin wax with the soap employed.

2. An emulsion in water and soap of a

compound wax comprising paraffin wax and a hard wax.

3. The method of making emulsions of compound waxes comprising paraffin and a relatively hard and high melting wax, which consists in melting a preponderant proportion of paraffin wax with a hard wax 30 to form the compound wax and then heating the wax mixture with soap and a quantity of water appropriate to the emulsification of the paraffin wax with the soap employed.

4. An emulsion in water and soap of a compound wax comprising a preponderant proportion of paraffin wax and a hard wax in subordinate proportion.

Signed by me at Boston, Massachusetts, 40 this 15th day of July, 1915.

GEORGE WELLINGTON MILES.

Witnesses:

ROBERT CUSHMAN,

CHARLES D. WOODBERRY.